

G. J. B. CHETWYND.  
MANUFACTURE OF STEEL.  
APPLICATION FILED JAN. 2, 1914.

1,211,545.

Patented Jan. 9, 1917.

7 SHEETS—SHEET 1.



Minister:  
Sillie E. Harrow  
March 2000

1,211,545.

G. J. B. CHETWYND.  
MANUFACTURE OF STEEL.  
APPLICATION FILED JAN. 2, 1914.

Patented Jan. 9, 1917.

7 SHEETS—SHEET 2.



Witness:  
Sister E. H. Knott  
M. F. Ridge

1,211,545.

G. J. B. CHETWYND.  
MANUFACTURE OF STEEL.  
APPLICATION FILED JAN. 2, 1914.

Patented Jan. 9, 1917.

7 SHEETS—SHEET 3.

Fig. 3.



Fig. 4.



Inventor

Godfrey John Boyle Chetwynd  
By Davis & Davis  
Attorneys

Witnesses:  
Lillian E. Harris  
A. M. Bridges

G. J. B. CHETWYND.  
MANUFACTURE OF STEEL.  
APPLICATION FILED JAN. 2, 1914.

1,211,545.

Patented Jan. 9, 1917.

7 SHEETS—SHEET 4.

Fig. 5



Fig. 9



Witnesses:  
S. E. Morris  
Godfrey John Boyle

Godfrey John Boyle  
Chas. Davis & Davis  
By Davis & Davis  
Attorneys

1,211,545.

G. J. B. CHETWYND,  
MANUFACTURE OF STEEL,  
APPLICATION FILED JAN. 2, 1914.

Patented Jan. 9, 1917.

7 SHEETS—SHEET 5.

Fig. 6.



Fig. 7.



Inventor

Witnesses:

Lillian E. Hensel  
M. J. Bridges

George John Boyle  
M. Davis & Davis  
Attorneys

1,211,545.

G. J. B. CHETWYND,  
MANUFACTURE OF STEEL,  
APPLICATION FILED JAN. 2, 1914.

Patented Jan. 9, 1917.

7 SHEETS—SHEET 6.

Fig 11.



Fig 10.



Inventor.

Patricia  
Sue E. Harris  
W.B. Bishop

Godfrey John Boyle  
By Davis & Davis  
Attorneys <sup>Chitenge</sup>

1,211,545.

G. J. B. CHETWYND.  
MANUFACTURE OF STEEL.  
APPLICATION FILED JAN. 2, 1914.

Patented Jan. 9, 1917.  
7 SHEETS-SHEET 7.



Inventor

Witnesses  
Sally E. Nease  
W. R. Bridges

Godfrey John Boyle Chetwynd  
By Davis & Davis  
Attorneys.

# UNITED STATES PATENT OFFICE.

GODFREY JOHN BOYLE CHETWYND, OF WEST RIDING, ENGLAND.

## MANUFACTURE OF STEEL.

1,211,545.

Specification of Letters Patent.

Patented Jan. 9, 1917.

Application filed January 2, 1914. Serial No. 809,972.

To all whom it may concern:

Be it known that I, GODFREY JOHN BOYLE CHETWYND, a subject of the King of Great Britain and Ireland, residing in the West Riding of Yorkshire, England, have invented Improvements in or Relating to the Manufacture of Steel, of which the following is a specification.

In tapping steel and iron from open hearth and other furnaces into ladles preparatory to running it into ingot or other molds, some slag is unavoidably drawn off with the steel or the iron (hereinafter included in the term steel) and owing to the impetus with which the molten stream falls into the ladle, becomes so intermingled with the steel in the ladle that it has not time to separate completely therefrom and rise to the surface thereof before the steel must be run off into the ingot or other molds before undue chilling of the steel in the ladle occurs. Consequently, in the manufacture of articles of various kinds made from such steel it is often found that the articles contain so much slag and other impurities that they have to be discarded, frequently after considerable work has been done thereon, thereby incurring considerable loss of time and money and reducing the output of salable articles.

Now the object of this invention is to enable articles made of steel to be produced of better and more reliable quality throughout.

For this purpose, molten steel with admixed slag, produced by any process, after being tapped from any open hearth or other steel or iron melting, making or refining furnace or vessel (hereinafter included in the term furnace) into a suitable receptacle in which it forms a deep bath and before it is run off therefrom into ingot or other molds is maintained in such a liquid condition by the aid of an electric current passing through the depth of the bath and for such a time, as to enable slag and other impurities, including gases, in the molten steel, to separate therefrom and rise to the surface thereof, and also to enable the purified steel to be still run from the bottom or lower part of the receptacle, while in a sufficiently liquid condition, into the molds as to produce sound ingots or castings, so that articles made from such purified steel, being

practically free from slag and other impurities or defects, shall be of more reliable quality throughout.

In carrying out the invention there is passed through the molten steel in the receptacle above referred to, as soon as may be, a current of electricity of sufficient strength to maintain the steel at the required temperature or even to increase the temperature thereof. For this purpose the bottom of the receptacle is provided with suitable conducting material to form one or more electrodes or poles suitably shaped and adapted for ready connection to and disconnection from an electric circuit. The opposite electrode or pole or electrodes or poles may be formed by one or more suitably shaped plates, rods or equivalent of suitable conducting material adapted to be readily placed in such position relatively to the molten metal that upon closing the electric circuit to which the electrodes or poles are connected an electric current will be caused to pass through the molten steel, substantially throughout its depth, either maintaining the temperature thereof approximately constant, or it may be, raising it, while the slag and other impurities, including gases, in the molten steel are allowed to separate therefrom and rise to the surface thereof, after which the purified steel is run off from the bottom or lower portion of the receptacle into a suitable mold or molds or other receptacle. The electrodes can be variously constructed and be variously adapted to be electrically connected up for use and the lower ones instead of passing through the bottom of the receptacle may be passed through the side or sides thereof close to the bottom; or one or more of them may be passed through the bottom of the receptacle and another or others through the side or sides of the receptacle and close to the bottom thereof. The receptacle may be an ordinary steel casting ladle or any other vessel, movable or stationary, in which a considerable depth of molten steel in relation to its horizontal cross section can be maintained during the treatment thereof so as to allow of the slag and other impurities rising to the top of the steel but it is essential that the latter can be subsequently run off from the bottom or lower portion of the receptacle, it may

be through a lateral tap hole or spout, into a casting ladle or through a bottom nozzle direct into molds without liability of the slag and other impurities again becoming intermixed therewith during the running off. This feature is essential to retaining the steel in the purified condition obtained by the treatment described. The receptacle may have a lining of ordinary refractory material, such as fireclay, constituting an acid lining. In all cases it is preferred to make the junction between the bottom and inner sides of the receptacle of curved shape.

In carrying out the treatment above referred to it is found advantageous first to cover the molten mass of steel in the receptacle with a thick layer of slag, say for example of a thickness of several inches, which can readily be obtained from the furnace from which the steel is obtained or from other suitable source, and which owing to its nature, will quickly become solidified in so far at least as its upper surface is concerned, so that the molten metal becomes protected against atmospheric effects during the purifying treatment, the electric current used passing through the slag. In some cases, as when a layer of slag of sufficient thickness and resistance is not available, an electric arc or arcs is or are produced between the electrode or electrodes and the molten mass of steel to prevent contact between these parts and to insure the presence of sufficient resistance in the electric circuit. The receptacle may have a suitable cover fitted to it but ordinarily it is preferred to dispense with a cover.

In the accompanying illustrative drawings, Figures 1 and 2 show respectively in side elevation and plan, one arrangement of plant suitable for carrying the invention into practice and wherein two receptacles are used, namely one in which the purifying treatment is carried out and the other, an ordinary casting ladle, into which the purified steel is run and thence run into molds. In Fig. 1, the stationary support and associated parts for one side of the receptacle are removed. Fig. 3 shows partly in side elevation and partly in vertical section, Fig. 4 in plan, with one half of the brick lining removed and Fig. 5 in side elevation taken at right angles to Fig. 3, the receptacle in which the purification process is carried out, and associated parts, shown to a smaller scale in Figs. 1 and 2. Figs. 6 and 7 show respectively in side elevation and plan, an alternative arrangement of receptacle and associated parts and Figs. 8, 9, and 10 are similar views to Figs. 3, 4 and 5 respectively of the receptacle used in such arrangement. Fig. 11 is a detail view, showing to a larger scale, one of the lower electrodes used in the receptacle. Fig.

12 is a diagram showing one arrangement of electrical connections that may be used.

In the example shown in Figs. 1 to 5 inclusive, 1 is a receptacle having an acid lining 2, say of fireclay, and external brackets 3 whereby it can be carried by horizontal supports 4, such as girders, arranged at opposite sides of a pit 5. Extending through the bottom of the receptacle 1 and its lining 2 are electrodes 6 made of iron rods that are connected together by horizontal conductors 7 in the form of strip copper, to similar connecting strips 8 the upper bent ends 8<sup>a</sup> of which serve as contacts arranged to bear upon other contact strips 9 carried by the upper surfaces of the supports 4, so that when the receptacle 1 is in position for use, the contact parts 8<sup>a</sup> and 9 will be subjected to the weight of the receptacle and its contents whereby good electrical connection will be made between them. Thin sheets of good conducting material of a soft nature, for example lead, may be placed between the contact parts 8<sup>a</sup> and 9 to further insure good electrical connection. In the example, there are a number of electrodes 6 spaced apart and extending through the bottom of the ladle 1. Each electrode may conveniently be made as shown in Fig. 3 and to a larger scale in Fig. 11, and comprises an iron rod the inner end portion 6 of which may advantageously be for about five inches of its length of small enough diameter, say of about eleven sixteenths of an inch, to allow the electric current used to raise its temperature to the melting point. The outer portion 6<sup>a</sup> of the electrode which is of greater diameter is adapted to be screwed into a rod 6<sup>b</sup> of still greater diameter, the part 6<sup>a</sup> having a squared portion 6<sup>c</sup> to admit of its being easily held while being screwed into place or removed for renewal. The part 6<sup>b</sup>, constituting an enlarged extension of the part 6, 6<sup>a</sup> of the electrode is made as a metal bolt arranged to be fixed in metal distance washers or sleeves 6<sup>d</sup>, 6<sup>e</sup> at the bottom of the ladle as shown. Or the whole electrode could be made one piece. The two sets of contact strips 9 are connected by suitable conductors 10, 10<sup>a</sup> (see Fig. 12), each to one end of the secondary windings 11 or 11<sup>a</sup> of two separate single phase transformers of which 12 and 12<sup>a</sup> are the respective primary windings. 13, 13<sup>a</sup> are two upper electrodes conveniently of graphite, fixed respectively in separate holders 14, 14<sup>a</sup> carried by but insulated from separate vertically adjustable supports 15, 15<sup>a</sup> by which the said electrodes can be moved into and out of position for use in the receptacle 1. For this purpose each support 15, 15<sup>a</sup> may, as in the example, be mounted to slide vertically on a frame 17, being carried by a rope 18, or equivalent, 130

led around suitably arranged guide pulleys 19 to a winch barrel 20 by suitable operation of which the position of the lower end of each upper electrode 13 or 13<sup>a</sup> can be readily adjusted to suit requirement. Automatic adjustment may be used if desired. The frame 17, in the example, is mounted to turn about a vertical axis so that the upper electrodes 13, 13<sup>a</sup>, when raised above the receptacle 1, can be readily turned into and out of position for use. The said upper electrodes 13 and 13<sup>a</sup> are respectively connected by copper conductors 21 and 21<sup>a</sup>, which are flexible where necessary, to the other or opposite ends of the secondary windings 11 and 11<sup>a</sup> of the two transformers to which the lower electrodes 6 are connected. The two ends *a* and *f* of the primary winding 12 are arranged to be respectively connected to one, namely 22, of the outer conductors 22, 23 and to the inner conductor 24 of a two phase three wire feeder by an oil switch 25, a throw over switch 26 and an isolating or main switch 27 through a meter 28. The two ends of the primary winding 12<sup>a</sup> of the other transformer are arranged to be similarly connected to the other outer conductor 23 and the inner conductor 24 of the feeder by a switch 25<sup>a</sup> and the throw over and isolating switches 26 and 27 through a meter 28<sup>a</sup>. Each primary winding 12, 12<sup>a</sup> may have a number of intermediate tap points, as shown at *b*, *c*, *d* and *e*, whereby the active length 35 of the primary winding 12 or 12<sup>a</sup> and consequently the voltage generated in the corresponding secondary winding 11 or 11<sup>a</sup> can be varied to suit requirement. In the example, the point *e* is arranged to be connected to the inner conductor 24 through the throw over switch 26 and one or other of the remaining tap points, namely *d* in the example, is arranged to be connected to the corresponding outer conductor 22 or 23 by a separate oil switch 25<sup>b</sup> or 25<sup>c</sup>. The switches 25, 25<sup>a</sup>, 25<sup>b</sup> 25<sup>c</sup> and 26 are or may be interlocked so that switch 26 must be closed before or opened after the others and when switches 25 and 25<sup>a</sup> are closed switches 25<sup>b</sup> and 25<sup>c</sup> must remain open or vice versa. 29 and 30 are single phase ammeter meters for indicating the currents in the respective secondary circuits; 31 an ammeter meter to indicate the resultant current in the neutral of the secondary circuits; 32 a power factor indicator; 33 a volt meter; 34 a recording ammeter and 35 a recording volt meter, these meters being arranged to be connected up for use in any suitable way such as that shown.

In the arrangement shown in Figs. 1 to 5, the receptacle 1 in which a charge of steel is to be treated, is provided with a lateral tap hole or spout 36 through which the molten steel, after being purified, is run off into an

ordinary casting ladle 37 supported for example from a crane. In the alternative arrangement shown in Figs. 6 to 10, the receptacle 1 is shown as provided with ordinary discharge nozzles 38 at the bottom 70 through which the purified steel can be run direct into a mold or molds.

Sometimes the electrical connections 7 connected to the lower electrodes 6 are adapted to bear directly upon metal conducting strips that are carried by girders at the bottom of the pit 5 and connected to the secondary current supply conductors 10, 10<sup>a</sup>, the upper electrodes 13, 13<sup>a</sup> being arranged and connected up as hereinbefore described 80 with reference to Figs. 1, 2 and 12.

It is found important to make the diameter of the upper ends of the lower iron electrodes 6, where they extend through the refractory lining of the ladle, of relatively small diameter as hereinbefore described, in order that the current density passing through them during the purification process, as hereinafter described, shall not fall appreciably below about 1250 amperes per square inch so that the said upper ends of the lower electrodes shall become melted. The result of this is that as the metal of the electrodes in the molten state will offer greater electrical resistance than when it is 95 in the solid state, the necessary resistance in the electric circuit will not be limited only to the slag on the surface of the molten metal, and there is provided in the lower portions of the molten mass of steel in the neighborhood of the bottom electrodes, areas of intense heat that will facilitate the heating of the whole mass of steel. As a consequence it is found that a steadier action on the molten steel is obtained, on the passage of the 100 electric current therethrough, than would be the case if lower electrodes of large sectional area were used. Furthermore, as a consequence of this steadier action, undesirable contact between the molten metal and the upper electrodes, by upheaval of metal due to too violent agitation therein, which would lead to short circuiting and its disadvantages, is minimized. Also, it is found advantageous to use during the greater part of the 110 purification process, current of relatively low voltage, that is to say not exceeding about 65 volts and it may with advantage be even less than this, as a greater and more regular heating of the mass of molten steel 120 is then found to take place than is the case when a higher voltage is used.

Into the receptacle 1 in each case a charge of molten steel in the normally finished state in which it has heretofore been cast into ingot or other molds is run from a furnace and a thick layer of slag, say of about six to ten inches in thickness may be run into the receptacle upon the top of the molten steel, after which the upper electrodes are brought 125 130

into position for use and electric current caused to pass through the slag and mass of molten steel.

With arrangements such as shown in the drawings good results have been obtained as follows:—About forty tons of molten steel in the normally finished state and obtained from an ordinary acid lined Siemens Martin open-hearth furnace was run into an ordinary acid lined receptacle of circular shape having a mean internal diameter of about 6 feet and an internal depth of about nine feet, the receptacle being provided at the bottom with ten vertical iron electrodes 6 of the kind hereinbefore referred to and shown in Figs. 3 and 11, that were connected, as hereinbefore mentioned, to one end of the secondary windings 11, 11<sup>a</sup> of the two transformers each of which was adapted to 15 produce a difference of potential varying from about 65 to 110 volts (see Fig. 12). The molten steel was covered with a layer of slag of about six to ten inches in thickness which immediately became solidified 20 on the surface as the top of the receptacle was open to the atmosphere. The two upper electrodes 13, 13<sup>a</sup> of graphite spaced about three feet six inches apart from center to center, each having a diameter of about 25 eight inches and connected to the opposite ends of the secondary windings 11, 11<sup>a</sup> as described, were then brought into contact with the solidified slag and the primary windings 12, 12<sup>a</sup> of the transformers supplied with 30 current from a two phase alternating current supply of 2200 volts and a periodicity of 60  $\frac{1}{2}$  per second, the secondary current produced and supplied to the electrodes 6 and 13, 13<sup>a</sup> having a voltage at the commencement of the treatment of about 80 volts, being later on altered to about 65 volts. The current passing melted the surface of 35 the slag in proximity to the upper electrodes and these electrodes were caused to descend into the slag until the passage of a steady current of the desired amount took place namely, in the example now being described, of about 3400 amperes per phase at the beginning, rising to about 4200 amperes per 40 phase on change of voltage, the current passing through slag between the upper electrodes and the molten steel. The current was maintained in action for about twenty minutes after it became steady, which took 45 place after about ten minutes from the commencement of the supply of current, and the molten steel, after the treatment thereof, was run off from the bottom of the receptacle into the second receptacle 37 from which it 50 was run into molds. In other instances the steel has been treated in an ordinary casting ladle fitted as shown in Figs. 8, 9 and 10 and run direct from that through bottom nozzles into the molds.

55 During the treatment above described,

frequent slight explosions took place in close proximity to the upper electrodes and in addition considerable expulsion of gas occurred, occasionally of such volume as to raise the solidified surface of the slag until the latter burst and released the gas. At other times on the solidified surface of the slag being perforated, the gas escaping under the influence of considerable pressure, burnt with a brilliant flame, at times varying very considerably in color.

Steel produced by the process above described is found to be improved in quality as compared with steel not so treated, and to be remarkably free from injurious impurities, gases and slaggy inclosures, this being due to the above described treatment and to the fact that after such treatment the steel was run off from the bottom of the ladle in which it was treated in such a manner that no slag was brought away with it. Moreover the cost of treating steel in the manner described is very small, the treatment of forty tons of steel in the above example being effected with an expenditure of about 245 Board of Trade units.

What I claim is:—

1. The process of purifying steel that has been normally finished in a steel making, refining or melting furnace and transferred to a receptacle so as to form therein a deep bath of molten metal preparatory to casting, which consists in causing electric current of large amperage to flow substantially through the whole depth of the molten metal and produce at the bottom thereof a small localized center of intense heat, maintaining the current to enable impurities to separate from the molten metal and rise to the surface thereof and afterward running off the purified metal from the bottom of the receptacle.

2. The process of purifying steel that has been normally finished in a steel making, refining or melting furnace and transferred to a receptacle so as to form therein a deep bath of molten metal preparatory to casting, which consists in causing electric current of large amperage to flow substantially through the whole depth of the molten metal and produce a number of separate centers of intense heat disposed over the bottom of the receptacle and in contact with the molten metal therein, maintaining the current to enable impurities to separate from the molten metal and rise to the surface thereof and afterward running off the purified metal from the bottom of the receptacle.

3. The process of purifying steel that has been normally finished in a steel making, refining or melting furnace and transferred to a receptacle so as to form therein a deep bath of molten metal preparatory to casting, which consists in causing electric cur-

rent of large amperage to flow substantially through the whole depth of the molten metal and produce a number of separate liquid centers of intense heat located at the bottom of the receptacle and in contact with the molten metal therein, maintaining the current to enable impurities to separate from the molten metal and rise to the surface thereof and afterward running off the purified metal from the bottom of the receptacle.

4. The process of purifying steel that has been normally finished in a steel making, refining or melting furnace and transferred to a receptacle so as to form therein a deep bath of molten metal preparatory to casting which consists in causing electric current of large amperage to flow substantially through the whole depth of the molten metal and produce at the bottom thereof a zone of intense heat in contact with the molten metal, maintaining the current to enable impurities to separate from the molten metal and rise to the surface thereof and afterward running off the purified metal.

5. The process of purifying steel that has been normally finished in a steel making, refining or melting furnace and transferred to a receptacle so as to form therein a deep bath of molten metal preparatory to casting which consists in causing electric current of large amperage to flow substantially through the whole depth of the molten metal

and produce at the bottom thereof a liquid center of intense heat in contact with the molten metal, maintaining the current to enable impurities to separate from the molten metal and rise to the surface thereof and afterward running off the purified metal from the bottom of the receptacle.

6. The process herein described of purifying steel that has been normally finished in a steel making, refining or melting furnace and transferred therefrom to a receptacle so as to form therein a deep bath of molten metal preparatory to casting, which consists in first covering the said bath of metal with a layer of slag and then causing an electric current to flow through said slag covering and substantially through the whole depth of the bath of metal and produce at the bottom thereof a zone of intense heat in contact with the molten metal, maintaining the current to enable impurities to separate from the molten metal and rise to the surface thereof and afterward running off the purified metal from the bottom of the receptacle.

Signed at 10 New Court, Lincoln's Inn, London, England, this twenty-second day of December, 1913.

GODFREY JOHN BOYLE CHETWYND.

Witnesses:

WILLIAM CROSS,  
FREDERICK WILLIAM PARTON BROUHAM.

Copies of this patent may be obtained for five cents each, by addressing the "Commissioner of Patents,  
Washington, D. C."